

1

3,809,532

**PROCESS FOR DYEING FIBRE MIXTURES OF POLYESTER AND WOOL**

Heinz Abel, Reinach, Basel-Land, Switzerland, assignor to Ciba-Geigy AG, Basel, Switzerland  
No Drawing. Continuation of abandoned application Ser. No. 849,859, Aug. 13, 1969. This application July 7, 1972, Ser. No. 269,652

Claims priority, application Switzerland, Aug. 16, 1968, 12,364/68

Int. Cl. D06p 3/82

U.S. Cl. 8—21 C

8 Claims

**ABSTRACT OF THE DISCLOSURE**

Mixture of polyester fibres and wool are dyed simultaneously with disperse dyestuffs and wool dyestuffs in the presence of sodium o-phenylphenolate, a levelling agent, and a wool reserve agent. The sodium o-phenylphenolate promotes the penetration of the disperse dyestuff into the polyester fibres and the other additives prevent demixing of the o-phenylphenolate carrier.

This is a continuation of application Ser. No. 849,859, filed Aug. 13, 1969, now abandoned.

The present invention relates to a process for dyeing fibre mixtures of polyesters and wool, with the polyester portion being dyed with dispersion dyestuffs and the wool being dyed with wool dyestuffs and in the presence of o-phenylphenol as a carrier in baths to which an aqueous stable carrier preparation is added in addition to the dyestuffs. The process is characterized in that the carrier preparation contains (a) the sodium salt of o-phenylphenol, (b) a levelling agent and (c) a wool reserve agent which has affinity for the fibre, with the quantity ratio (a):(b):(c) lying in the range of (20 to 60):(5 to 20):(2 to 20) and with the dyebath containing 2 to 15%, relative to the material to be dyed, of the sodium salt of o-phenylphenol.

Particularly suitable aqueous carrier preparations are those containing (a) the sodium salt or potassium salt of o-phenylphenol, (b) at least one addition compound of 5 to 70 mols of ethylene oxide to monoamines or diamines, with at least one nitrogen atom of the amine being substituted by a hydrocarbon residue having 16 to 22 carbon atoms, as a levelling agent, and (c) at least one condensation product of formaldehyde and (a') sulphones which possess two phenol residues bonded to the  $\text{SO}_2-$  groups or (b') hydroxybenzenesulphonic or naphthalenesulphonic acids as a wool reserve agent having affinity for the fibre, with the quantity ratio (a):(b):(c) lying in the range (20 to 60):(5 to 20):(2 to 20) and with the dyebath containing 2 to 15%, relative to the material to be dyed, of the sodium or potassium salt of o-phenylphenol.

It is known to use ortho-phenylphenol and para-phenylphenol as carriers for dyeing polyester material or material containing polyesters. These carriers are intended to promote the penetration of the dyestuff and better complete dyeing of the polyester fibre, since, as the polyesters lack functional groups and their ability to swell in water is only slight, dyeing with normal dyebaths in most cases does not produce usable results.

When using prefabricated carrier preparations as auxiliary agents for dyeing polyester material care must be taken that the carrier dispersion does not demix or that a constituent crystallizes out. These disadvantages occur in the case of all known carrier preparations which contain ortho-phenylphenol and thus these preparations can only be added to the goods to be dyed when the preparations are in the form of an emulsion or solution, for which special measures, for example boiling the preparation, are

2

in most cases necessary. On cooling such emulsions the ortho-phenylphenol again crystallizes out.

It has now been found that an aqueous carrier preparation which in addition to o-phenylphenol as the actual carrier contains a levelling agent and a wool reserve agent having affinity for the fibre is stable at room temperature also and can be directly added to the dyebath without further pretreatment.

According to the invention, wool and fibre material from polyesters are dyed simultaneously. These fibre materials can for example be present in mixing ratios of 40:60 to 60:40 and in the most diverse processing conditions, for example in a loose form, as combed tops, yarn or a mixed woven fabric.

In this process wool is dyed with wool dyestuffs which can be reactive or non-reactive towards the substrate to be dyed and which can belong to the most diverse classes of dyestuffs, especially classes of the acid azo and anthraquinone dyestuffs, but also of the azomethine dyestuffs.

20 The chromium and cobalt complexes of monoazo dyestuffs which contain more than one molecule of dyestuff per atom of metal bound as a complex, with at least one dyestuff molecule being free of sulphonate acid groups and of carboxylic acid groups not participating in the complex formation, prove to be particularly advantageous. The heavy metal atom can be bonded to two mutually different or two identical dyestuff molecules. The complex-forming group of the dyestuffs can for example be a o-hydroxy-o'-aminoazo grouping, a o-hydroxy-o'-carboxyazo grouping or preferably an o,o'-dihydroxyazo grouping.

25 By reactive dyestuffs there are to be understood those dyestuffs which can enter a chemical, that is to say covalent, bond with the material to be dyed. These dyestuffs for example contain ethyleneimide, epoxy, vinyl, vinylsulphonic or acrylic acid groups or halogenated groups such as  $\alpha,\beta$ -dibromopropionic acid,  $\beta$ -chloropropionic acid,  $\alpha$ - or  $\beta$ -bromacrylic acid residues or monohalogenated or dihalogenated triazinyl and pyrimidyl residues, as reactive groups.

30 35 40 The polyester fibres are dyed with disperse dyestuffs. These dyestuffs can be dyed onto hydrophobic fibres from aqueous dispersion and can belong to the most diverse classes of dyestuffs, with azo and anthraquinone dyestuffs deserving particular consideration.

45 The levelling agents which are employed in the carrier preparation are for example the polyglycol-ether derivatives, which are in themselves known, of long-chain hydroxyl compounds such as, say, the castor oil acid residues of castor oil, or of monoamines and diamines, with at least one nitrogen atom being substituted by the hydrocarbon residue of a long-chain fatty acid; furthermore these adducts can also be quaternized at a nitrogen atom or be esterified with a polybasic acid at the end of a polyglycol chain, or be both quaternized and esterified.

50 55 60 As starting substances, single higher-molecular alkylamines or also amine mixtures, such as are obtained on conversion of natural fatty acid mixtures, for example tallow fatty acid, into the corresponding amines are used. Amines with 16 to 22 carbon atoms to which 5 to at most 70 mols of ethylene oxide have been added are suitable. The following may be mentioned individually as amines: hexadecylamine, octadecylamine, arachidylamine



65 behenylamine  $\text{CH}_3(\text{CH}_2)_{21}-\text{NH}_2$ , octadecenylamine and N-alkylpropylenediamines with the appropriate hydrocarbon residues.

70 75 The wool reserve agents are colorless compounds having affinity for the fibre are for example water-soluble condensation products of formaldehyde and mixtures of

(a) sulphones possessing two phenol residues, which may have further substituents, bonded to the  $\text{SO}_2-$  group, and (b) monocyclic hydroxyarylsulphonic acids or bicyclic arylsulphonic acids. Advantageously, mixtures are used in which the molecular quantity ratio of (a) sulphone to (b) sulphonic acid is 30:70 to 85:15.

However, the individual components of the mixtures of sulphones and sulphonic acids, such as for example water-soluble condensation products of formaldehyde and sulphones which possess two phenol residues, which may have further substituents, bonded to the  $\text{SO}_2-$  group, or hydroxybenzene-sulphonic acids or naphthalenesulphonic acids, are however also suitable.

Both the sulphones and the sulphonic acids and also their reaction products with formaldehyde are compounds which are in themselves known.

Amongst the sulphones, the dihydroxydiphenylsulphones of formula



are preferred, wherein  $\text{R}_1$  and  $\text{R}_2$  independently of one another denote hydrogen atoms, methyl groups or sulphonic acid groups. Phenolsulphonic acids and cresolsulphonic acids may be mentioned as examples of the monocyclic hydroxyarylsulphonic acids.

The condensation of the mixtures with formaldehyde is appropriately carried out in an aqueous alkaline medium. For example, a mixture of a sulphone and a sulphonic acid of the nature indicated in water can be rendered alkaline with sodium or potassium hydroxide, formaldehyde added (for example 0.9 to 1.1 mols per mol of mixture of hydroxyaryl compounds) and the whole kept at an elevated temperature for a prolonged period, for example 5 to 6 hours. Mixtures of sulphones and sulphonic acids can also be manufactured by reacting a hydroxybenzene such as phenol, p-cresol or a xylanol, with concentrated sulphuric acid. Thereafter, when the requisite quantity of alkali hydroxide has been added to establish the alkaline medium following the addition of water, the condensation with formaldehyde can be carried out without an intermediate separation. A condensation under acid conditions, for example in acetic acid solution, is also possible.

In addition to the mixtures of sulphone and sulphonic acid which have been mentioned, the condensation products of formaldehyde with the diarylsulphones of the above-mentioned nature which possess at least one phenolic hydroxyl group are also suitable to be used by themselves as a reserve agent.

The limits of the components mentioned for the aqueous carrier preparation lie between 20 to 60 parts of orthophenylphenol, 5 to 20 parts of a levelling agent and 2 to 20 parts of a wool reserve agent having affinity for the fibre, with the difference from 100 parts optionally being made up with water. A clear solution of low viscosity which gives an alkaline reaction is obtained.

The amount of carrier preparation which is added to the dyebath is 10 to 40% relative to the weight of the material to be dyed. The dyebath should react acid during the dyeing process, and the pH-value should be about 5; the requisite acid reaction is achieved by adding low molecular organic acids, especially formic acid and acetic acid. Following the dyeing process, the goods are appropriately further treated for a short time with a dyebath rendered alkaline with ammonia and adjusted to pH 8, and are then rinsed and dried.

The advantages of the present process reside in the stability, which is good at room temperature also, and hence in the easy manipulation of the carrier preparation which is directly added to the dyebath without prior dissolution. Furthermore the preparation improves the dispersion stability of the dispersion dyestuffs so that no separate addition of a dispersing agent to the dyebath is

necessary. The action of the reserve agent having affinity for the fibre resides in the fact that on each kind of fibre it is the dyestuff intended for the particular fibre which is predominantly absorbed, as a result of which both fibres are dyed in the same shade if suitable dyestuffs are used simultaneously, or that when using wool and dispersion dyestuffs of different colors in the same dyebath a two-color effect can be achieved. Additionally however, the reserve agent also serves as a dispersing agent for the dispersion dyestuffs, and at the same time it counteracts the dyestuff retention capacity of the levelling agent for the wool dyestuffs, which in the amount used would otherwise be too great for a usable dyeing still to be obtained. The levelling agent in the carrier preparation serves as an emulsifier for the actual carrier, the o-phenylphenol, but then also acts as a dispersing agent in the dyebath for the dispersion dyestuffs and naturally as a levelling agent for the wool dyestuffs.

The present process for dyeing fibre mixtures of wool and polyester fibres now has the advantage that in addition to the dyestuff a stable aqueous carrier preparation is added to the dyebath, the auxiliary agent combination of the carrier preparation being on the one hand a dispersing agent and emulsifier for the actual carrier but on the other hand also a levelling agent for the dyestuffs of the dyebath, with one of the components additionally acting as a wool reserve agent, so that a uniform tone-on-tone dyeing can be achieved.

In the manufacturing instructions which follow, and in the examples, the parts denote parts by weight and the percentages denote percentages by weight unless otherwise stated.

#### MANUFACTURING INSTRUCTION FOR THE CARRIER PREPARATION

|                                             | Parts |
|---------------------------------------------|-------|
| Sodium salt of o-phenylphenol               | 50    |
| One of the levelling agents described below | 10    |
| Reserve agent described below               | 10    |
| Water                                       | 30    |
|                                             | 100   |

are stirred together at 50 to 60° C. Thereafter the mixture is slowly cooled to room temperature.

##### (1) Levelling agents

(a) 5% strength aqueous solution of the ammonium salt of the acid sulphuric acid ester of the adduct of 1 mol of a tallow fatty amine (consisting of 30% hexadecylamine, 24% octadecylamine and 45% octadecenylamine) with 7 mols of ethylene oxide, quaternized with chloracetamide and having the formula



wherein R denotes the hydrocarbon residue of the tallow fatty amine and  $(m+n)$  has an average value of 7.

(b) 50% strength aqueous solution of a mixture of (1) an adduct of 1 mol of tallow fatty amine and 20 mols of ethylene oxide, quaternized with dimethylsulphate and (2) the ammonium salt of the acid sulphuric acid ester of the adduct of 1 mol of a fatty amine (consisting of 10% stearylamine, 55% arachidylamine and 35% behenylamine) and 30 mols of ethylene oxide.

(c) 30% strength aqueous solution of an adduct of 1 mol of a fatty amine (having a hydrocarbon residue of 18 to 22 carbon atoms) and 30 mols of ethylene oxide.

(d) 50% strength aqueous solution of an adduct of 1 mol of a fatty amine (having a hydrocarbon residue of 18 to 22 carbon atoms) and 30 mols of ethylene oxide, quaternized with dimethyl sulphate.

(e) 50% strength aqueous solution of an adduct of 1 mol of a fatty amine (having a hydrocarbon residue of 16 to 20 carbon atoms) and 70 mols of ethylene oxide.

(f) 50% strength aqueous solution of the ammonium salt of the acid sulphuric acid ester of the adduct of 1 mol of tallow fatty amine and 30 mols of ethylene oxide.

(g) 50% strength aqueous solution of the ammonium salt of the acid sulphuric acid ester of the adduct of 1 mol of the reaction product of oleic acid and propylenediamine, in which one amino group possesses the hydrocarbon residue corresponding to that of soya fatty acid, with 10 mols of ethylene oxide.

(h) 50% strength aqueous solution of the sodium salt of the trisulphosuccinic acid ester of the adduct of castor oil and 40 mols of ethylene oxide.

(i) 30% strength aqueous solution of an adduct of 1 mole of oleylamine and 8 mols of ethylene oxide.

(2) Reserve agent

(a) 35% strength aqueous solution of a condensation product of formaldehyde and a mixture of 4,4'-dihydroxydiphenylsulphone - 3 - sulphonic acid and o-cresol-4-sulphonic acid, which has been adjusted to a pH-value of 7 with 30% strength sodium hydroxide solution (molar ratio of sulphone to sulphonic acid, 40:60).

(b) 35% strength aqueous solution of the condensation product (a), with a molar ratio of sulphone to sulphonic acid of 80:20.

(c) 35% strength aqueous solution of a condensation product of formaldehyde and 4,4' - dihydroxydiphenylsulphone - 3 - sulphonic acid, which has been adjusted to a pH-value of 7 with 30% strength sodium hydroxide solution.

(d) 35% strength aqueous solution of a condensation product of formaldehyde and a mixture of 4,4' - dihydroxy - 3 - methyl diphenylsulphone and 1-hydroxy-2-methylbenzene - 4 - sulphonic acid (molar ratio of sulphone to sulphonic acid, 40:60). Similar condensation products are obtained if 4,2'-dihydroxy-diphenylsulphone, 4,4' - dihydroxy - 3,3' - dimethyl-diphenylsulphone or mixtures of these sulphones with 1-hydroxy - 2 - methylbenzene - 4 - sulphonic acid or phenol - 4 - sulphonic acid are reacted with formaldehyde in the indicated manner.

(e) 50% strength aqueous solution of a condensation product of formaldehyde and a mixture of naphthalene-sulphonic acid and 4,4'-dihydroxydiphenylsulphone.

(f) Condensation product of naphthalenesulphonic acid and formaldehyde.

(g) 50% strength aqueous solution of a condensation product of formaldehyde and 4,4' - dihydroxydiphenylsulphone - 3 - sulphonic acid which has been adjusted to a pH-value of 7 with 50% strength sodium hydroxide solution.

(h) 35% strength aqueous solution of a condensation product of phenolsulphonic acid and formaldehyde, which has been adjusted to a pH-value of 7.8 with 30% strength sodium hydroxide solution.

(i) 35% strength aqueous solution of a condensation product of 4,4' - dihydroxydiphenylsulphone and formaldehyde, which has been adjusted to a pH-value of 7.5 with 30% strength aqueous sodium hydroxide solution.

(k) 35% strength aqueous solution of a condensation product of formaldehyde and a mixture of phenolsulphonic acid, 4,4' - dihydroxydiphenylsulphone and 2-naphthol - 6 - sulphonic acid, which has been adjusted to a pH-value of 7.5 with 30% strength aqueous sodium hydroxide solution (molar ratio phenolsulphonic acid to 4,4'-dihydroxydiphenylsulphone to 2-naphthol - 6 - sulphonic acid, 50:50:10).

In addition to the above-mentioned parts of the individual components for the preparation of the carrier, all variations within the limits mentioned are of course also possible which comprise 20 to 60 parts of the sodium salt of o-phenylphenol, 5 to 20 parts of the levelling agent and 2 to 20 parts of the wool reserve agent having affinity for the fibre.

EXAMPLE 1

A woven fabric consisting of 55% polyester and 45% wool is washed, treated in the kier and pre-set for 30 seconds at 180° C.

100 kg. of this woven fabric are introduced into 4000 litres of water at 60° C. The following additives are then introduced into the bath: 8000 g. of ammonium sulphate, 4000 g. of 85% strength formic acid, 20,000 g. of the carrier preparation as described in the manufacturing instruction, using the levelling agent (1)-(a) and the reserve agent (2)-(a), 1000 g. of the dyestuff of formula



and 800 g. of the dyestuff of formula



30 The pH-value should be about 5.

The dyeing temperature is raised to 92-96° C. within 40 minutes and dyeing is carried out for 90 minutes at this temperature. The bath is then cooled to 80° C. and adjusted to a pH-value of 8 with ammonia, and the goods are treated for 20 minutes at 80° C., then rinsed warm and cold, and if desired acid-treated with 1% of 85% strength formic acid.

A fast blue dyeing with good matching of the shades of the two kinds of fibre results. Instead of the indicated components for the preparation of the carrier, it is also possible to use the remaining products indicated in the manufacturing instruction, such as for example (1)-(b) and (2)-(d) or (1)-(d) and (2)-(f).

EXAMPLE 2

100 kg. of woven fabric consisting of 55% polyester and 45% wool are pre-wetted in 4000 litres of water at 60° C. on a winch. 8000 g. of ammonium sulphate and 3000 g. of 85% strength formic acid are then added. After distributing these additives, 25,000 g. of the carrier preparation as described in the manufacturing instruction, using the levelling agent (1)-(a) and the reserve agent (2)-(b), 1200 g. of the dyestuff of formula



and 800 g. of the dyestuff of formula



are further added to the bath. The pH-value of the bath is adjusted to 4.5-5.5.

The bath is then warmed to the boil within 40 minutes and dyeing is carried out for 90 minutes at this temperature. Thereafter the bath is cooled to 80° C. and adjusted to a pH-value of 8 with ammonia, and the goods are further treated for 20 minutes, rinsed and dried. A fast level blue dyeing of both kinds of fibre results. Instead of the indicated components for the preparation of the carrier, it is also possible to use the remaining products indicated in the manufacturing instruction.

## EXAMPLE 3

100 kg. of cheeses consisting of 55% polyester and 45% wool are wetted in 2000 litres of water at 60° C. in a cheese dyeing apparatus. The following are then added: 4000 g. of ammonium sulphate, 3000 g. of 85% strength formic acid, 20,000 g. of the carrier preparation as described in the manufacturing instruction, using the levelling agent (1)-(c) and the reserve agent (2)-(b), 500 g. of the dyestuff of formula

(5)



250 g. of the dyestuff of formula

(6)



180 g. of the dyestuff of formula

(7)



and 100 g. of the dyestuff of formula

(8)



The pH-value of the dyebath is adjusted to 4.5-5.5. The temperature is raised to 106° C. within 45 minutes and dyeing carried out for 50 minutes at this temperature. Thereafter the dyebath is cooled and the goods are rinsed and dried.

A level fast yellow dyeing of both fibre portions results.

Instead of the indicated components for the preparation of the carrier, it is also possible to use the remaining products indicated in the manufacturing instruction.

## EXAMPLE 4

100 kg. of yarn consisting of 55% polyester fibres and 45% wool, are dyed in a cheese dyeing apparatus in the following manner

The yarn is introduced into 1500 litres of water at 60° C. The following additives are then introduced into the bath: 3000 g. of ammonium sulfate, 6000 g. of acetic acid (80% strength) and 9000 g. of the carrier preparation consisting of: 50 parts of the potassium salt of o-phenylphenol, 10 parts of levelling agent (1)-(i), 10 parts of the reserve agent (2)-(a) and 30 parts of water. The pH-value is adjusted to 4.5 with acetic acid.

The following dyestuffs are then added: 2000 g. of the dyestuff of formula

5



10

1000 g. of the dyestuff of formula

15



20

1450 g. of the dyestuff of formula

25



30



35



40



45



50



The bath is then warmed to 103° C. within 45 minutes and dyeing is carried out for 40 minutes at this temperature.

The bath is then cooled to 80° C., the pH-value increased to 8 with ammonia, and the goods treated in this bath for 20 minutes. They are then rinsed and dried. A fast red dyeing with good matching of the shade on both fibre portions results.

Similar good results are obtained if carrier preparations are used which contain the levelling agents (1)-(e), (f) and (i) and the reserve agents (2)-(e), (g) and (k).

## EXAMPLE 5

100 kg. of woven fabric of 55% polyester and 45% wool are warmed to 60° C. in 4000 litres of water in a winch tank. The following additives are then introduced into the bath: 8000 g. of ammonium sulphate, 6000 g. of 85% strength formic acid, and 5000 g. of the carrier preparation of the following composition: 40 parts of the sodium salt of o-phenylphenol, 15 parts of levelling agent (1)-(a), 15 parts of reserve agent (2)-(a) and 30 parts of water. The pH-value of the bath is adjusted to pH 5 with formic acid. The following dyestuffs are then added: 1000 g. of the dyestuff of formula

(13)



and 1500 g. of the dyestuff of formula

(14)



The bath is warmed to a high temperature within 45 minutes and dyeing is carried out for 60 minutes at this temperature. Thereafter the goods are rinsed and post-washed in a fresh bath at 80° C. as follows:

Bath additives: 2 g./l. of 85% strength formic acid and 2 g./l. of the leveling agent (1)-(b).

Time: 30 minutes.

Thereafter the goods are rinsed and dried. A fast dyeing with a two-color effect results, the polyester fibre being dyed blue whilst the wool is dyed red.

Equally good results are obtained if instead of the indicated carrier preparation the following carrier preparations are used:

(1) 30 parts of the sodium salt of o-phenylphenol, 10 parts of levelling agent (1)-(b), 15 parts of reserve agent (2)-(a) and 45 parts of water.

(2) 50 parts of the sodium salt of o-phenylphenol, 10 parts of levelling agent (1)-(a), 10 parts of reserve agent (2)-(f) and 30 parts of water.

(3) 50 parts of the sodium salt of o-phenylphenol, 10 parts of levelling agent (1)-(f), 10 parts of reserve agent (2)-(h) and 30 parts of water.

(4) 50 parts of the sodium salt of o-phenylphenol, 10 parts of levelling agent (1)-(i), 10 parts of reserve agent (2)-(h) and 30 parts of water.

What is claimed is:

1. A process for simultaneously dyeing fibre mixtures of polyesters and wool, wherein the polyester portion is dyed with dispersion dyestuffs and the wool with wool dyestuffs in the presence of o-phenylphenol as a carrier, which comprises adding to the dyebath containing said dyestuffs from 10 to about 40% of the weight of material being dyed of a carrier preparation comprising

(a) 20 to about 60% of the sodium or potassium salt of o-phenylphenol,

(b) 5 to about 20% of a levelling agent comprising the addition product of 5 to 70 mols of ethylene oxide to monoamines or diamines, with at least one nitrogen atom of the amine being substituted by an alkyl radical having 16 to 22 carbon atoms and wherein at least one nitrogen atom is quaternized and at least one polyglycol chain is esterified with a polybasic acid, and

(c) 2 to 20% of a wool reserve agent comprising the condensation product of formaldehyde, and (a') sulphones which possess two hydroxy phenyl groups bonded to the SO<sub>2</sub>- group, or (b') hydroxybenzenesulphonic or naphthalene-sulphonic acids,

wherein the ratio (a):(b):(c) is in the range (20 to

75 8—25, 26, 89, 173

60):(5 to 20):(2 to 20), and wherein the dyebath contains 2 to 15% of the sodium or potassium salt of o-phenylphenol, relative to the weight of material being dyed.

5 2. Process according to claim 1 in which the dyeing is carried out at 90 to 110° C.

10 3. Process according to claim 1 in which the levelling agents consist of a mixture of an addition compound having at least one quaternized nitrogen atom and an addition compound having at least one polyglycol chain which is esterified by a polybasic acid.

15 4. Process according to claim 1 in which the carrier preparation is added to the dyebaths which contains, as the wool reserve agent having affinity for the fibre, condensation products of formaldehyde and mixtures of (a') sulphones which possess two phenol residues bonded to the SO<sub>2</sub>- group and (b') hydroxybenzenesulphonic or naphthalenesulphonic acids.

20 5. Process according to claim 4 in which the hydroxybenzenesulphonic acids of component (b') are phenol-sulphonic and cresolsulphonic acids.

25 6. Process according to claim 1 in which a carrier preparation is added to the dyebaths which contain, as a wool reserve agent having affinity for the fibre condensation products of formaldehyde and sulphones of formula



30 wherein R<sub>1</sub> and R<sub>2</sub> independently of one another denote hydrogen atoms, methyl groups or sulphonic acid groups.

35 7. Process according to claim 4 characterized in that the molecular quantity ratio of (a') sulphone condensation product to (b') sulphonic acid condensation product in the reserve agent is 30:70 to 85:15.

40 8. A stable aqueous carrier preparation according to claim 1 which comprises (a) the sodium or potassium salt of o-phenylphenol, (b) at least one addition compound of 5 to 70 mols of ethylene oxide to monoamines or diamines, with at least one nitrogen atom of the amine being substituted by an alkyl radical of 16 to 22 carbon atoms, as a levelling agent and (c) at least one condensation product of formaldehyde and (a') sulphones which possess two hydroxy phenyl groups bonded to the SO<sub>2</sub>- group and/or (b') hydroxylbenzene-sulphonic or naphthalenesulphonic acids, as a wool reserve agent having affinity for the fibre, with the quantity ratio (a):(b):(c) lying in the range (20 to 60):(5 to 20):(2 to 20) and with the dyebath containing 2 to 15%, relative to the material to be dyed, of the sodium or potassium salt of o-phenylphenol.

#### 55 References Cited

##### UNITED STATES PATENTS

|           |        |                  |       |         |
|-----------|--------|------------------|-------|---------|
| 2,999,731 | 9/1961 | Harding          | ----- | 8—54    |
| 3,097,040 | 7/1963 | Casty            | ----- | 8—54    |
| 3,097,047 | 7/1963 | Weinstein et al. | ----- | 8—94    |
| 3,528,761 | 9/1970 | Keller et al.    | ----- | 8—172 X |

##### OTHER REFERENCES

Cheetham: Dyeing Fiber Blends, 1966, p. 283.  
Diserens: Vol. II, Chem. Tech. Dye. and Print., 1951, p. 78.

65 Bird: Theory and Practice of Wool Dyeing, 1963, pp. 177-179.

Trotman: Dye. and Chem. Tech. of Tex. Fibers, 1964, pp. 523-524.

70 HERBERT B. GUYNN, Primary Examiner  
B. H. HESS, Assistant Examiner